

Nov. 16, 1954

G. F. NADEAU ET AL

2,694,639

LIGHT-SENSITIVE METAL BASE PHOTOGRAPHIC ELEMENT

Filed June 14, 1951

**Fig. 1**



**Fig. 2**



**Fig. 3**



*Gale F. Nadeau  
Clemens B. Starck  
Carl F. Smith*  
INVENTORS

*BY Daniel J. Mayne  
W.H.W. Dowell*

ATTY. & AGT.

# United States Patent Office

2,694,639

Patented Nov. 16, 1954

1

2,694,639

## LIGHT-SENSITIVE METAL BASE PHOTOGRAPHIC ELEMENT

Gale F. Nadeau, Clemens B. Starck, and Carl F. Smith, Rochester, N. Y., assignors to Eastman Kodak Company, Rochester, N. Y., a corporation of New Jersey

Application June 14, 1951, Serial No. 231,632

10 Claims. (Cl. 95—8)

This invention relates to light-sensitive photographic elements and more particularly to such elements having a metallic base or support.

In the art of photography, it is well known that the conventional hydrophilic colloid-silver halide emulsion layers require a support such as cellulose ester, resin, paper, metal, etc. Many patents directed to means for adhering the emulsions to such supports have been granted mainly in the field of adhering emulsions to cellulose ester and resin supports.

The prior art would indicate that relatively few problems have arisen when the emulsion is to be adhered to metallic supports. However, we have discovered that in order to obtain optimum adherence and quality in metal-based sensitive elements, it is essential to provide certain adhesive or subbing layers for obtaining the desired adherence of the emulsion to the metal support. This is particularly true when the sensitive elements are to be subjected to abnormal atmospheric conditions such as high temperature and low relative humidity, with conditions are manifest by the formation of fissures in the emulsion layer.

Accordingly, the primary object of our invention is to provide subbing layers for adhering hydrophilic colloid-silver halide emulsion layers to metal supports. Other objects will become apparent from consideration of the following description of our invention.

In general, the objects of our invention are accomplished by providing a metal base or support, such as aluminum, steel, copper, brass, etc., particularly in the form of thin sheets, with two thin subbing layers, the first comprising a mixture of a light-colored inert filler material, a resinous copolymer, and preferably, but not necessarily, polyvinyl acetate, the second layer being a mixture of polyvinyl acetate and cellulose nitrate. Thus provided with a subbed metal-based element, the desired hydrophilic colloid-silver halide emulsion layer may then be adhered thereto by means of one or more additional organic colloid subbing layers containing polymeric units in common with the colloid vehicle comprising the particular hydrophilic organic colloid-silver halide emulsion vehicle under consideration.

In the drawings:

Fig. 1 shows in greatly enlarged cross-sectional view the appearance of metal-based photographic element carrying a gelatino-silver halide emulsion layer adhered to the metal base by means of the subbing layers of the invention.

Fig. 2 is a similar view of a metal-based element carrying a polyvinyl alcohol-silver halide emulsion layer adhered to the base by means of the novel subbing layers.

Fig. 3 is a similar view of a metal-base film utilizing the subbing layers of the invention for causing adherence of a cellulose acetate-silver halide emulsion to the metal support.

The following examples illustrate preferred methods for adhering hydrophilic organic-colloid-silver halide emulsion layers to metal supports:

### Example 1

A first thin subbing layer is applied to an aluminum support by conventional methods from a solution of the following composition:

|                    | Per cent |
|--------------------|----------|
| Polyvinyl acetate  | 4        |
| Resinous copolymer | 4        |
| Titanium oxide     | 3        |

2

| Per cent      |
|---------------|
| Acetone       |
| Butyl acetate |

5 In this subbing composition the solvents may be replaced by a comparable amount of methylene chloride, but the indicated solvent combination is preferred. In the composition the ratio of the two resins may be varied somewhat, but approximately equal parts by weight of the  
10 two resins are preferred. However, as previously mentioned, this composition can include only the solid ingredients: resinous copolymer and filler material. The polyvinyl acetate is not an essential ingredient, serving only as a modifier or plasticizer. The essence of the invention is the use of the copolymer and filler material as the first subbing layer 11 in conjunction with the second subbing layer 12 of polyvinyl acetate and cellulose nitrate to be described hereinafter. The filler material, titanium oxide, can be varied within reason, a range of from about  
15 25 to 75 per cent by weight of the resins of the filler material being most efficacious. The filler material, titanium oxide, is representative of a class of light-colored inert materials such as barium sulfate, calcium carbonate, zinc oxide, etc., essential to successful operation  
20 of our invention. That is, it has been found that while useful products can be made when the filler material is omitted from the subbing formula, the filler material, when used in conjunction with the resinous vehicle, not only provides a white or light-colored background for silver images developed on the metal support, but, which is more important, prevents flow of the subbing layers during drying and shrinking of the emulsion, thus preventing the emulsion from showing shrinkage cracks or skidding. In the formula the viscosity of the  
25 30 particular polyvinyl acetate used is not especially critical as it appears only to alter the viscosity of the subbing composition.

The resinous copolymer indicated in the subbing formula is a carboxylated copolymer of a mixture of vinyl chloride, vinyl acetate, and an  $\alpha,\beta$ -ethylenically unsaturated dicarboxylic acid, such as fumaric or maleic acid, preferably one containing about 86 per cent by weight of vinyl chloride groups, about 13 per cent by weight of vinyl acetate groups, and about 1 per cent by weight of maleic acid groups. In the various figures of the drawings is shown the position of the subbing layer 11 affixed to the metal support 10 by the method just described.

The first subbing layer 11 is then coated with the  
50 second thin subbing layer from the following representative composition:

| Per cent                         |
|----------------------------------|
| Cellulose nitrate                |
| Polyvinyl acetate                |
| Titanium oxide                   |
| Acetone                          |
| Ethylene glycol monomethyl ether |
| Methyl alcohol                   |

60 In the various figures of the drawings this subbing layer is represented by layer 12.

In the subbing formula immediately above, the filler material may be omitted, but its presence tends to improve the appearance of the coating. The type of cellulose nitrate used is not especially critical, but it is preferable to use the well known low to medium viscosity highly alcohol-soluble variety containing about 11 per cent nitrogen. The proportions of polyvinyl acetate and cellulose nitrate in the formula may be varied somewhat, the preferred proportions being from about six to twelve parts of cellulose nitrate per part of polyvinyl acetate.

As pointed out above, the metal support, now having been provided with the two subbing layers of the invention, can be sensitized with a variety of organic hydrophilic colloid-silver halide emulsions. This is accomplished by utilizing a third intervening subbing layer having approximately the same chemical and physical characteristics as the colloid vehicle of the emulsion layer.

Accordingly, a gelatino silver halide emulsion is applied to the element provided with subbing layers 11 and 12 as follows:

A third thin subbing layer 13 was applied to the surface of subbing layer 12 from the composition:

|                     | Per cent |
|---------------------|----------|
| Gelatin             | 1.2      |
| Methyl alcohol      | 87.8     |
| Water               | 10       |
| Glacial acetic acid | 1.0      |

in which the gelatin concentration may be varied as desired, for example, between 1 and 2 per cent concentration. Following this, a gelatino-silver halide emulsion layer 14 of the conventional type was coated over subbing layer 13. The result was a film of good flexibility free of the mentioned defects. As will be apparent, suitable antihalation materials, for example, dyes, may be incorporated into the sensitive film as desired.

#### Example 2

As shown in Fig. 2, the metal support 10 such as aluminum, steel, etc., is provided with the subbing layers 11 and 12, layer 11 containing modifier or not in the manner of Example 1, following which a layer of partially hydrolyzed polyvinyl acetate is applied thereto to cause adherence of a polyvinyl alcohol-silver halide emulsion layer 17 to the support. Preferably, this is accomplished by coating successively on layer 12 subbing layers 15 and 16 from the following compositions, respectively:

|                                  | Per cent |
|----------------------------------|----------|
| Hydrolyzed polyvinyl acetate     | 1.5      |
| Cellulose nitrate                | 0.5      |
| Ethylene glycol monomethyl ether | 15       |
| Methyl alcohol                   | 75       |
| Water                            | 8        |

In this formula the ratio of partially hydrolyzed polyvinyl acetate to cellulose nitrate can be varied somewhat, for example, within the range of from about two to six parts per part of cellulose nitrate. The hydrolyzed polyvinyl acetate used in the above formula contained 37.9% vinyl acetate groups by weight, the remainder being vinyl alcohol groups. While a hydrolyzed polyvinyl acetate of this analysis is preferred, other hydrolyzed polyvinyl acetates varying as much as 10 per cent in vinyl alcohol group content can be used for the same purpose.

|                                                          | Per cent |
|----------------------------------------------------------|----------|
| Polyvinyl alcohol                                        | 1.5      |
| Methyl alcohol                                           | 40       |
| Zirconium nitrate (based on weight of polyvinyl alcohol) | 5        |
| Water                                                    | 54       |

Following application of subbing layer 16, a polyvinyl alcohol-silver halide emulsion layer 17 is coated in a well known manner to provide the finished product shown in Fig. 2 of the drawings.

#### Example 3

The pre-subbed element prepared as described in Example 1 and having subbing layers 11 and 12 of the invention on the metal support 10, layer 11 preferably containing the modifier resin polyvinyl acetate, is coated as shown in Fig. 3 with a subbing layer 18 from the composition

|                                  | Per cent |
|----------------------------------|----------|
| Hydrolyzed cellulose ester       | 1-3      |
| Water                            | 10       |
| Ethylene glycol monomethyl ether | 15       |
| Methyl alcohol                   | 74       |

The hydrolyzed cellulose ester used in the above composition is selected from hydrolyzed cellulose esters containing from about 19 to 33% acyl groups, and preferably consists of hydrolyzed cellulose acetate containing about 27% acetyl. Hydrolyzed cellulose esters described in the Salo U. S. Patent 2,110,491 granted March 8, 1938, are suitable for this composition and for the colloid vehicle of the silver halide emulsion layer 19 which is subsequently applied over layer 18. The cellulose ester emulsion layer can be applied from solvent systems selected from those disclosed in the patent mentioned.

We claim:

1. A light-sensitive photographic element comprising a metal support, adhered directly thereto, a first layer of a mixture of a light-colored inert filler material and a resinous copolymer of a mixture of vinyl chloride, vinyl

acetate and an  $\alpha,\beta$ -ethylenically unsaturated dicarboxylic acid, said layer being substantially free of polymerizable material adhered directly to said first layer a second layer of a mixture of polyvinyl acetate and cellulose nitrate, and a hydrophilic organic colloid-silver halide emulsion layer adhered to said second layer.

2. A light-sensitive photographic element comprising a metal support, adhered directly thereto, a first layer of a mixture of a light-colored inert filler material, polyvinyl acetate and a resinous copolymer of vinyl chloride, vinyl acetate and an  $\alpha,\beta$ -ethylenically unsaturated dicarboxylic acid, said layer being substantially free of polymerizable material, adhered directly to said first layer a second layer of a mixture of polyvinyl acetate and cellulose nitrate, and a hydrophilic colloid-silver halide emulsion layer adhered to said second layer.

3. A light-sensitive photographic element comprising a metal support, adhered directly thereto, a first layer of a mixture of a light-colored inert filler material, polyvinyl acetate and a resinous copolymer containing about 86% by weight of vinyl chloride groups, about 13% by weight of vinyl acetate groups, and about 1% by weight of maleic acid groups, said layer being substantially free of polymerizable material, adhered directly to said first layer a second layer of a mixture of polyvinyl acetate and cellulose nitrate, and a hydrophilic organic colloid-silver halide emulsion layer adhered to said second layer.

4. A light-sensitive photographic element comprising a metal support, adhered directly thereto, a first layer of a mixture of a light-colored inert filler material, polyvinyl acetate and a resinous copolymer containing about 86% by weight of vinyl chloride groups, about 13% by weight of vinyl acetate groups, and about 1% by weight of maleic acid groups, said layer being substantially free of polymerizable material, adhered directly to said first layer a second layer of a mixture of polyvinyl acetate and cellulose nitrate, and a gelatino-silver halide emulsion layer adhered to said second layer by means of a gelatin layer.

5. A light-sensitive photographic element comprising a metal support, adhered directly thereto, a first layer of a mixture of a light-colored inert filler material, polyvinyl acetate and a resinous copolymer containing about 86% by weight of vinyl chloride groups, about 13% by weight of vinyl acetate groups, and about 1% by weight of maleic acid groups, said layer being substantially free of polymerizable material, adhered directly to said first layer a second layer of a mixture of polyvinyl acetate and cellulose nitrate, and a polyvinyl alcohol-silver halide emulsion layer adhered to said second layer by means of a layer of partially hydrolyzed polyvinyl acetate.

6. A light-sensitive photographic element comprising a metal support, adhered directly thereto, a first layer of a mixture of a light-colored inert filler material, polyvinyl acetate and a resinous copolymer containing about 86% by weight of vinyl chloride groups, about 13% by weight of vinyl acetate groups, and about 1% by weight of maleic acid groups, said layer being substantially free of polymerizable material, adhered directly to said first layer a second layer of a mixture of polyvinyl acetate and cellulose nitrate, and a polyvinyl alcohol-silver halide emulsion layer adhered to said second layer by means of a hydrophilic cellulose ester layer.

7. A light-sensitive photographic element comprising a metal support, adhered directly thereto, a first layer of a mixture of approximately equal parts by weight of polyvinyl acetate and a resinous copolymer containing about 86% by weight of vinyl chloride groups, about 13% by weight of vinyl acetate groups and about 1% by weight of maleic acid groups together with from about 25-75% by weight of resin of a light-colored inert filler material, said layer being substantially free of polymerizable material, adhered directly to said first layer a second layer of a mixture of from about 6 to 12 parts of cellulose nitrate per part of polyvinyl acetate, and a gelatino-silver halide emulsion layer adhered to said second layer by means of a gelatin layer.

8. A light-sensitive photographic element comprising an aluminum support, adhered directly thereto, a first layer of a mixture of approximately equal parts by weight of polyvinyl acetate and a resinous copolymer containing about 86% by weight of vinyl chloride groups, about 13% by weight of vinyl acetate groups and about 1% by weight of maleic acid groups, together with from about 25-75% by weight of resin of a light-colored inert filler material, said layer being substantially free of poly-

merizable material, adhered directly to said first layer a second layer of a mixture of from about 6 to 12 parts of cellulose nitrate per part of polyvinyl acetate, and a gelatino-silver halide emulsion layer adhered to said second layer by means of a gelatin layer.

9. A light-sensitive photographic element comprising a metal support, adhered directly thereto, a first layer of a mixture of approximately equal parts by weight of polyvinyl acetate and a resinous copolymer containing about 86% by weight of vinyl chloride groups, about 13% by weight of vinyl acetate groups and about 1% by weight of maleic acid groups together with from about 25-75% by weight of resin of a light-colored inert filler material, said layer being substantially free of polymerizable material, adhered directly to said first layer a second layer of a mixture of from about 6 to 12 parts of cellulose nitrate per part of polyvinyl acetate, a third layer of a mixture of from about 2 to 6 parts of partially hydrolyzed polyvinyl acetate per part cellulose nitrate adhered directly to said second layer, and a polyvinyl alcohol-silver halide emulsion layer adhered to said third layer by means of a layer of polyvinyl alcohol.

10. A light-sensitive photographic element comprising a metal support, adhered directly thereto, a first layer of a mixture of approximately equal parts by weight of polyvinyl acetate and a resinous copolymer containing about 86% by weight of vinyl chloride groups, about 13% by

weight of vinyl acetate groups and about 1% by weight of maleic acid groups together with from about 25-75% by weight of resin of a light-colored inert filler material, said layer being substantially free of polymerizable material, adhered directly to said first layer a second layer of a mixture of from about 6 to 12 parts of cellulose nitrate per part of polyvinyl acetate, and a hydrophilic cellulose organic acid ester-silver halide emulsion layer adhered to said second layer by means of a layer of 10 hydrolyzed cellulose organic acid ester of approximately 19 to 33% acyl content.

#### References Cited in the file of this patent

#### UNITED STATES PATENTS

|    | Number    | Name          | Date          |
|----|-----------|---------------|---------------|
| 15 | 2,362,580 | Nadeau et al. | Nov. 14, 1944 |
|    | 2,398,056 | Staud         | Apr. 9, 1946  |
|    | 2,411,590 | Powell        | Nov. 26, 1946 |
| 20 | 2,483,465 | Johnson       | Oct. 4, 1949  |
|    | 2,527,263 | Hart          | Oct. 24, 1950 |
|    | 2,569,954 | Ruebensaal    | Oct. 2, 1951  |

#### FOREIGN PATENTS

|    | Number  | Country       | Date          |
|----|---------|---------------|---------------|
| 25 | 600,039 | Great Britain | Mar. 30, 1948 |